

Patented June 20, 1933

1,914,990

# UNITED STATES PATENT OFFICE

WILLIAM J. BURR, OF TOLEDO, OHIO, ASSIGNOR TO TOLEDO SCALE MANUFACTURING COMPANY, OF TOLEDO, OHIO, A CORPORATION OF NEW JERSEY

## MATERIAL FOR BEARINGS, KNIFE EDGES, AND THE LIKE

No Drawing.

Application filed May 16, 1930. Serial No. 453,105.

This invention has for its object the production of improved bearings, knife edges and the like.

Another object is the provision of a rust-resistant material having a very hard wear-resistant surface.

Another object is the provision of a material having a very hard, thin case and a core of a hardness substantially equal to that of tempered steel.

Another object is the production of a process for obtaining metal for bearings, knife edges and the like having the characteristics mentioned above.

Other objects and advantages will be apparent from the following description.

In carrying out my process for making improved material and knife edge pivots, bearings and the like therefrom, I employ steel of substantially the following composition:

|           | Percent    |
|-----------|------------|
| Carbon    | .5 to .7   |
| Silicon   | .7 to .9   |
| Manganese | .5 to .7   |
| Chromium  | 7.5 to 8.5 |
| Tungsten  | 7.5 to 8.5 |

The remainder being iron, which may contain small amounts of impurities such as phosphorus, silicon and sulphur.

Specifically, I prefer to employ the following:

|           | Percent |
|-----------|---------|
| Carbon    | .60     |
| Silicon   | .80     |
| Manganese | .60     |
| Chromium  | 8.00    |
| Tungsten  | 8.00    |

The remainder being iron, which may contain small amounts of impurities such as phosphorus, silicon and sulphur.

This steel is first formed into the shape of the bearing, pivot or other part to be produced by any convenient method such as forging, rolling, drawing or machining. The formed pieces are then heated to a temperature of 2100 to 2200 degrees Farenheit and quenched in oil. They are then ground to remove all decarburization from the surfaces which are to be hardened. The pieces

so treated have a hardness of 600 to 650 when tested by the Brinnell machine and are very rust resistant.

In order to provide a wearing surface of great hardness, the pieces are next subjected to nitriding by being placed in a retort which is brought to a temperature of 975 to 1100 degrees Farenheit and through which a stream of ammonia gas is passed. The parts are kept in the retort and subjected to the influence of the ammonia gas for a period of one or more hours. Four hours' treatment results in the formation of a very thin, hard wear-resistant case. The pieces so treated will not exhibit any greater hardness when tested with the Brinnell machine than untreated pieces, but the surface cannot be braided by a file and is little affected even by long wear. The hardness of the case as determined by testing with a Vickers machine and the result converted by calculation into values according to the Brinnell system is from 900 to 1100. While pieces which have been treated do not exhibit any greater hardness under the Brinnell test than untreated pieces, on the other hand the core is not perceptibly softened by the heating to which it is subjected during the treatment with ammonia.

The embodiment of my invention herein described is to be regarded as illustrative only, and it is to be understood that the invention is susceptible to variation, modification and change within the spirit and scope of the subjoined claims.

Having described my invention, I claim:

1. An article of manufacture having a steel core of approximately the formula

|           | Percent    |
|-----------|------------|
| Carbon    | .5 to .7   |
| Silicon   | .7 to .9   |
| Manganese | .5 to .7   |
| Chromium  | 7.5 to 8.5 |
| Tungsten  | 7.5 to 8.5 |

The remainder being iron, which may contain small amounts of impurities such as phosphorus, silicon and sulphur,

and a surface hardened by treatment with ammonia at an elevated temperature.

2. An article of manufacture having a steel core of the formula

|                | Percent |
|----------------|---------|
| Carbon -----   | .60     |
| 5 Silicon----- | .80     |
| Manganese----- | .60     |
| Chromium-----  | 8.00    |
| Tungsten-----  | 8.00    |

10 The remainder being iron, which may contain small amounts of impurities such as phosphorus, silicon and sulphur,

and a surface hardened by treatment with ammonia at an elevated temperature.

WILLIAM J. BURR.

15

20

25

30

35